

## United States Patent Office

3,328,303

Patented June 27, 1967

1

3,328,303

PROCESS FOR PROTECTING GALVANIZED IRON  
AGAINST ATTACK BY STRONG ACIDS

Walter Mahnkopf, Mannheim, Germany, assignor to C. F. Boehringer & Soehne G.m.b.H., Mannheim-Waldhof, Germany, a corporation of Germany  
No Drawing. Filed July 23, 1964, Ser. No. 384,779  
Claims priority, application Germany, Sept. 14, 1963,  
B 73,525

9 Claims. (Cl. 252—79.4)

The present invention relates to a process of protecting galvanized iron against attack by strong acid and more particularly the invention relates to a process of protecting galvanized iron against attack by strong acid by incorporating in the acid treatment agent in addition to quinoidine a small amount of a quinoline derivative.

It is known that quinoidine, which is obtained as a by-product in the manufacture of quinine acts to curb the attack of strong acids upon various metals (DRP 548 315). The above-named compound has achieved considerable importance as a corrosion-inhibitor during the past few years and is marketed under the name "Brindi." However, it has been observed that the protective effect of the quinoidine is greatly diminished in those instances in which iron and zinc are simultaneously present so that they are both subject to the attack by the acid at the same time as for instance happens when the two metals are conductively interconnected. In such instances, as for example, in the case of galvanized iron, the zinc as an anode is preferentially attacked by the acid giving rise to the formation of corrosion elements. As a result, the galvanization of the iron (zinc coating) is dissolved within a relatively short period of time, whereupon the iron very rapidly undergoes corrosion and disintegration.

It is, therefore, an object of the present invention to provide a simple process of protecting galvanized iron against an attack by a strong acid utilizing quinoidine and a quinoline derivative as protective agent whereby the above-enumerated disadvantages and deficiencies of the final products are overcome.

It is a further object of the present invention to provide a process for protecting galvanized iron against attack by strong acids which process has the advantage that the result achieved by the use of the additional additive is considerably greater than could have been anticipated from the results achieved from either alone.

Other objects and advantages of the present invention will be apparent from the further reading of the specification and the appended claims.

In accordance with the invention it has now been found that the protection from acid of galvanized iron provided by incorporating quinoidine into the acid agents which come into contact with the same is considerably improved if there is additionally included in such agents a small amount of a quinoline derivative. In accordance with the invention it is preferable to use such quinolines as are condensed with and/or substituted by a benzene ring, as for example, acridine, phenanthridin, 7,8-benzoquinoline, 2-phenylquinoline, or 9-phenylacridine.

It is known that the speed of dissolution of metals may be inhibited by various simple quinoline derivatives, such as acridine (Zeitschrift fuer anorganische Chemie, 233/1937, page 236 et seq.). However, it has been established that the protective effect of these inhibitors is insufficient against the attack of acid upon galvanized iron. As illustrated by the following examples, if a combination of the aforementioned quinoline derivatives and quinoidine is used, the protective effect is markedly enhanced and is greater than could be expected from the effect of the individual components and is in fact a synergistic effect.

The following examples are given by way of illustration and not limitation:

2

## Example 1

A galvanized steel wire (40 mm. in length, diameter of 3.5 mm.) having a zinc coating of 16-17 $\mu$  was inserted into 1.33 N hydrochloric acid. The time required for 10% of the zinc coating to be dissolved was determined and in a similar manner the dissolution times with various inhibitor additives present was determined. The results are shown in the following table:

## TABLE

|                               | Dissolution of 10% of the zinc coating (seconds) |
|-------------------------------|--------------------------------------------------|
| 1.33 N hydrochloric acid:     |                                                  |
| Without any additive          | 45                                               |
| 0.2% quinoidine               | 110                                              |
| 0.1% acridine                 | 110                                              |
| 0.2% quinoidine+0.1% acridine | 840                                              |

## Example 2

The experiment described in Example 1 was repeated; however the dissolving bath contained 2 N hydrochloric acid and 2-phenylquinoline was substituted for the acridine. The following results were obtained:

|                                       | Dissolution of 10% of the zinc coating (seconds) |
|---------------------------------------|--------------------------------------------------|
| 2 N hydrochloric acid:                |                                                  |
| Without additive                      | 10                                               |
| 0.3% quinodine                        | 60                                               |
| 0.2% 2-phenylquinoline                | 210                                              |
| 0.3% quinodine+0.2% 2 phenylquinoline | 680                                              |

## Example 3

A galvanized steel wire (40 mm. long, 3 mm. diameter, 8.5 $\mu$  zinc coating) the ends of which had been coated with a layer of paraffin in order to eliminate as much as possible the formation of local elements (corrosion) along the ends of the wire was employed. The wire was inserted into 2 N hydrochloric acid and the time taken for 5% of the zinc coating to be dissolved determined in the absence of any additive as well as the additives as hereinafter set out.

|                                        | Dissolution of 5% of the zinc coating (seconds) |
|----------------------------------------|-------------------------------------------------|
| 2 N hydrochloric acid:                 |                                                 |
| Without additive                       | 12                                              |
| 0.3% quinodine                         | 65                                              |
| 0.1% 7,8-benzoquinoline                | 420                                             |
| 0.3% quinodine+0.1% 7,8-benzoquinoline | 1140                                            |

## Example 4

Example 3 was repeated, however, 9-phenylacridine was substituted for benzoquinoline. The ends of the wires were not coated with paraffin. The following results were obtained:

|                                      | Dissolution of 5% of the zinc coating (seconds) |
|--------------------------------------|-------------------------------------------------|
| 2 N hydrochloric acid:               |                                                 |
| Without additive                     | 5                                               |
| 0.3% quinodine                       | 30                                              |
| 0.3% 9-phenylacridine                | 8                                               |
| 0.3% quinodine+0.3% 9-phenylacridine | 570                                             |

## Example 5

A galvanized steel wire (40 mm. long, 3 mm. diameter) having a zinc coating of 10 $\mu$  was inserted into 2 N hydrochloric acid. The time for dissolution of 5% of the zinc coating was determined and in a similar manner there were determined the corresponding periods required when inhibitor-additives were present. The results are shown in the following table:

|                                   | Dissolution of 5% of the zinc coating (seconds) |
|-----------------------------------|-------------------------------------------------|
| 2 N hydrochloric acid:            |                                                 |
| Without additive                  | 6                                               |
| 0.3% quinodine                    | 51                                              |
| 0.2% phenanthridine               | 72                                              |
| 0.3% quinodine+0.2 phenanthridine | 192                                             |

Similar results as in the above shown examples, demonstrating the synergistic effect of quinoidine and a quinoline derivative are obtained by using sulfuric acid instead of hydrochloric acid.

The amount of quinoline derivatives can be varied from 0.05 to 2%, the preferred amount being from 0.1 to 0.5%. The amount of quinoidine can also be varied from 0.05 to 2%, the preferred amount being from 0.1 to 0.5%. The lower limits of amounts are given by the effectiveness of protection, the upper limits are given by the price of the products.

It is within the scope of this invention that further additives can be given to the acid solution such as surfactants and dyes. Preferred surfactants are those which are resistant to strong acids, such as alkylphenolpolyglycoether (for instance HOSTAPAL or ARKOPAL from "Farbwerke Hoechst" and LENSODEL from the "Shell Corp."). If desired, also indicator dyes can be added; i.e. pH-indicators for proving the effectiveness of the products.

What is claimed is:

1. In the process for protecting galvanized iron from attack of strong acids by incorporating 0.05 to 2% of quinoidine in said acid prior to the application thereof to the galvanized iron, the improvement of additionally incorporating in said acid 0.05-2% of a member selected from the group consisting of acridine, phenanthridine, 7,8-benzoquinoline, 2-phenylquinoline and 9-phenylacridine.
2. Improvement according to claim 1 which comprises incorporating 0.1-0.5% of said group member into said acid.
3. Improvement according to claim 1 wherein said strong acid is a member selected from the group consisting of hydrochloric and sulfuric acid.

4. A composition for protecting galvanized iron against attack from strong acid comprising a mixture of (A) quinoidine and (B) a member selected from the group consisting of acridine, phenanthridine, 7,8-benzoquinoline, 2-phenylquinoline and 9-phenylacridine in a ratio of A:B of 1-40:40-1.

5. A composition for protecting galvanized iron against attack from strong acid comprising a mixture of quinoidine and acridine in a ratio of 2:1.

6. A composition for protecting galvanized iron against attack from strong acid comprising a mixture of quinoidine and 2-phenylquinoline in a ratio of 3:2.

7. A composition for protecting galvanized iron against attack from strong acid comprising a mixture of quinoidine and 7,8-benzoquinoline in a ratio of 3:1.

8. A composition for protecting galvanized iron against attack from strong acid comprising a mixture of quinoidine and 9-phenylacridine in a ratio of 1:1.

9. A composition for protecting galvanized iron against attack from strong acid comprising a mixture of quinoidine and phenanthridine in a ratio of 3:2.

#### References Cited

##### UNITED STATES PATENTS

|    |           |         |                |       |             |
|----|-----------|---------|----------------|-------|-------------|
| 25 | 1,746,677 | 2/1930  | Rhodes         | ----- | 252-148     |
|    | 2,167,621 | 8/1939  | Beaver         | ----- | 252-148     |
|    | 2,499,283 | 2/1950  | Robinson       | ----- | 252-148     |
|    | 2,694,001 | 11/1954 | Hayes et al.   | ----- | 252-79.4    |
|    | 2,965,577 | 12/1960 | Heimann et al. | ----- | 252-148     |
|    | 3,135,632 | 6/1964  | Lucas et al.   | ----- | 252-79.4 XR |

ALEXANDER H. BRODMERKEL, Primary Examiner.

L. B. HAYES, Assistant Examiner.